

3,183,088

## PROCESS FOR FORMING IMAGES

Heman Dowd Hunt, Eatontown, N.J., assignor to E. I. du Pont de Nemours and Company, Wilmington, Del., a corporation of Delaware  
No Drawing. Filed Sept. 12, 1961, Ser. No. 137,534  
11 Claims. (Cl. 96—27)

This invention relates to a process of forming images in optically sensitized, light-developable, direct-writing radiation-sensitive elements.

It is known to latensify those photographic silver halide layers which are processed by liquid development by means of certain liquid baths. These baths comprise hydrogen peroxide, sodium perborate, potassium metabisulfite, soluble gold salts, solutions containing nitrosodisulfonate ions, etc. It is also known to latensify such liquid processed elements by means of gaseous treatment and by means of supplemental exposure. Latensification, of course, refers to the treatment of an exposed radiation-sensitive element after image exposure but before development.

In assignee's U.S. application Ser. No. 61,840, Patent No. 3,033,678, May 8, 1962, and application Ser. No. 852,190, Patent No. 3,033,682, May 8, 1962, there are described light-developable direct-writing radiation-sensitive elements suitable for oscilloscopic recording and similar uses which do not require liquid processing. These elements comprise novel silver halide emulsion layers containing an excess of water-soluble halide in an amount sufficient to provide an excess of halide ions over that necessary to precipitate all of the silver in the water-soluble silver salts as silver halide and a relatively large quantity of stannous salts based on the silver halide. These elements are quite sensitive in the blue and ultraviolet regions of the spectrum and they are exposed by either high pressure, mercury arc lamps, xenon lamps or any other source which is rich in blue and ultraviolet energy.

According to assignee's Hunt U.S. application Ser. No. 117,805, filed June 19, 1961, it has been found that the elements described therein, and above, which contain either a relatively high quantity (0.5 to 120 mole percent) of stannous salts alone or a relatively high quantity of the stannous salts in combination with 0.1 mole percent or more of plumbous salt can be optically sensitized to form novel photosensitive products. To be able to optically sensitize silver halide grains in the presence of a relatively large quantity of stannous salts, e.g. of the order of 10 mole percent based on silver halide, as taught in said application, is quite surprising considering the fact that the stannous salt is in operative association with the silver halide grains. The optically sensitized silver halide and emulsion layers of said application makes it possible to use various other sources of exposing radiation such as zirconium and tungsten lamps with attendant advantages.

The process of this invention comprises (a) exposing to image-forming radiation containing radiation in the region of normal sensitivity of a silver halide photographic emulsion and/or in the region of extended sensitivity conferred by the presence of an optical sensitizing dye, a washed, light-sensitive colloid-silver halide emulsion layer having an average grain size of 0.1 to 10 microns containing (1) 0.5 to 120 mole percent of a water soluble stannous salt, (2) a sensitizing amount of an optical sensitizing dye taken from the group consisting of cyanine, pseudocyanine, carbocyanine and merocyanine dyes capable of extending the sensitivity of a silver bromide emulsion from the normal blue region to at least one of the green, red and infrared regions of the spectrum, and having added thereto (3) at least one water-soluble halide taken from the group consisting of lithium, sodium, po-

tassium, calcium, magnesium and ammonium chloride, bromide and iodide in an amount sufficient to provide an excess of halide ions over that necessary initially to precipitate all of the silver as silver halide, (b) latensifying the element resulting from the image exposure of step (a) by irradiating said element for about 1 to about 60 seconds with light radiation in the region of greatest response in the region of extra sensitivity conferred to the silver halide emulsion by said dye, and (c) photodeveloping the latensified element by exposing it to actinic light (i.e., radiation containing wavelengths from 3000 to 5000 Å.) having an intensity less than the exposing radiation (a) for a period of at least 1 second. At room temperature, usually about 30 seconds are required to give an adequate visible image whereas at temperatures of 200°—300° F. a period of 1 second gives an adequate visible image. In general, there should be at least a 10% excess of halide ions present. Any photographic silver halide emulsion layer or elements embodying such a layer disclosed in application Ser. No. 117,805 can be used in the process of this invention. The exposure step (a) can be carried out for about 0.01 to about 10,000 microseconds.

In the examples which follow, the coated materials were tested by using a Mark III, Edgerton, Germen-shausen Grier, Inc. electronic flash sensitometer similar to that described by Wyckoff and Edgerton, Journal of the Society of Motion Picture and Television Engineers, 66, 474 (1957). This instrument uses a xenon discharge tube as a source of radiation. The exposure time was 10<sup>-5</sup> seconds. The radiation was modulated with a  $\sqrt{2}$  step tablet of 21 steps in the density range of 0.05 to 3.05. The latent image formed was latensified by yellow light attained by a yellow Wratten No. 8 filter modulation of white 40-watt fluorescent lights at 50 foot-candles intensity for a period of 5 seconds. Photo-development was then accomplished by removing the yellow filter and exposing the latensified element to white light for a period of several minutes to obtain maximum image density. With this type of development, an image of much higher density in the toe region of the sensitometric H and D<sup>1</sup> curve is obtained than has heretofore been possible. The latensified images may also be liquid developed, stabilized and fixed. The instant invention will be illustrated but is not intended to be limited to, the following detailed examples.

## Example I

A gelatino-silver chlorobromide emulsion washed to remove most of the chloride containing 100 milligrams per mole of silver bromide of 5,5'-dimethyl-3,3',9-triethyl benzselenazole carbocyanine iodide, 1 mole percent of plumbos nitrate, 10 mole percent of stannous chloride, and 30 mole percent excess bromide ions, all based on the silver halide, was made and coated in the manner described in Example I of assignee's Hunt U.S. application Ser. No. 117,805, filed June 19, 1961. The finished photographic element was exposed in the sensitometer described above to a 10<sup>-5</sup> sec. flash of the xenon lamp and then latensified by exposure for 5 seconds through a Wratten No. 8 (K-2) filter having good transmission from about 500 mu on into the infrared, to a 40-watt white fluorescent lamp at 50 foot-candles intensity. The filter was removed and the image was photodeveloped for 30 minutes under the above fluorescent lamp. The element was also exposed to blue light by means of a Wratten No. 47 filter, to green light by means of a Wratten No. 61 filter and to red light by means of a Wratten No. 29 filter. The results shown below are given as the number of steps made visible by the exposure through the  $\sqrt{2}$  step

<sup>1</sup> See: Mees, "The Theory of the Photographic Process," pages 591, 710 and 724, published by The Macmillan Co., New York [1946].

wedge. The letters W, B, G, R, K-2, D<sub>21</sub> and Δ indicates white light, blue light, green light, K-2 filter latensification, density at step 21 under white light exposure, and the difference between fog or back ground density and density at step 21. The figures shown under K-2 filter indicates the steps to be added to the number of steps under white light exposure which indicates the improvement in effective speed brought about by latensification. The exposure results are as follows.

| W  | B  | G | R  | K-2   | D <sub>21</sub> | Fog | Δ   |
|----|----|---|----|-------|-----------------|-----|-----|
| 17 | 12 | 8 | 13 | 5''+1 | .51             | .17 | .34 |

It will be seen that the latensification exposure through the K-2 filter for five seconds added one full  $\sqrt{2}$  density step to the white light exposure. In other words step 18 of the step wedge is made visible by the white light exposure with the latensification step.

#### Example II

Example I was repeated except that the emulsion contained 100 milligrams of the optical sensitizing dye: 3,3'-diethyl-9-methyl benzothiazole carbocyanine p-toluene sulfonate per mole of silver halide. All exposure conditions were carried out as described in Example I with the following results.

| W  | B  | G  | R | K-2   | D <sub>21</sub> | Fog | Δ   |
|----|----|----|---|-------|-----------------|-----|-----|
| 18 | 12 | 12 | 7 | 5''+1 | .55             | .21 | .34 |

#### Example III

Example I was repeated except that the emulsion contained 100 milligrams of the optical sensitizing dye: 5,5'-dibromo-3,3'-diethyl-9-methyl benzothiazole carbocyanine p-toluene sulfonate per mole of silver halide. All conditions of exposure were the same as described in Example I. The exposure results were as follows:

| W  | B  | G | R | K-2   | D <sub>21</sub> | Fog | Δ   |
|----|----|---|---|-------|-----------------|-----|-----|
| 17 | 12 | 9 | 9 | 5''+1 | .51             | .23 | .28 |

#### Example IV

Example I was repeated except that the emulsion contained 100 milligrams of the optical sensitizing dye: 5,5',9-trimethyl-3,3'-diethyl benzothiazole carbocyanine iodide. All exposure conditions were the same as those described in Example I with the following results:

| W  | B  | G  | R | K-2   | D <sub>21</sub> | Fog | Δ   |
|----|----|----|---|-------|-----------------|-----|-----|
| 17 | 13 | 11 | 9 | 5''+2 | .51             | .19 | .32 |

#### Example V

Example I was repeated except that the emulsion contained 100 milligrams of the optical sensitizing dye: 5,5'-diphenyl-9-methyl-3,3'-diethyl benzoxazole carbocyanine iodide per mole of silver halide. All conditions of exposure were the same as described in Example I with the following results.

| W  | B  | G  | R  | K-2   | D <sub>21</sub> | Fog | Δ   |
|----|----|----|----|-------|-----------------|-----|-----|
| 19 | 13 | 14 | -- | 5''+3 | .48             | .17 | .31 |

#### Example VI

Example I was repeated except that the emulsion contained 100 milligrams of the optical sensitizing dye: 5-methyl-3,1'-diethyl-2,2'-selenopseudocyanine iodide per mole of silver halide. All conditions of exposure were the same as described in Example I with the following results.

| W  | B  | G  | R  | K-2   | D <sub>21</sub> | Fog | Δ   |
|----|----|----|----|-------|-----------------|-----|-----|
| 17 | 13 | 11 | -- | 5''+2 | .51             | .20 | .31 |

#### Example VII

Example I was repeated except that the emulsion contained 100 milligrams of the optical sensitizing dye: 5,5'-dimethyl-3,3',9-triethyl benzothiazole carbocyanine iodide per mole of silver halide. All conditions of exposure were the same as described in Example I with the following results.

| W  | B  | G | R | K-2   | D <sub>21</sub> | Fog | Δ   |
|----|----|---|---|-------|-----------------|-----|-----|
| 17 | 12 | 8 | 9 | 5''+1 | .55             | .20 | .35 |

#### Example VIII

Example I was repeated except that the emulsion contained 100 milligrams of the optical sensitizing dye: 5,5'-dimethyl - 9 - phenyl - 3,3' - diethyl benzothiazole carbocyanine iodide per mole of silver halide. All conditions of exposure were the same as described in Example I with the following results.

| W  | B  | G | R | K-2   | D <sub>21</sub> | Fog | Δ   |
|----|----|---|---|-------|-----------------|-----|-----|
| 16 | 12 | 3 | 5 | 5''+1 | .53             | .22 | .31 |

#### Example IX

Example I was repeated except that the emulsion contained 50 milligrams of the merocyanine optical sensitizing dye: 3 - ethyl - 5 - [1 - ethyl - 2(1) - benzoxazolidene-isopropylidene] - 2 - thio - 2,4 - oxazole dione. All exposure conditions were the same as those described in Example I with the following results.

| W  | B  | G | R  | K-2   | D <sub>21</sub> | Fog | Δ   |
|----|----|---|----|-------|-----------------|-----|-----|
| 17 | -- | 7 | -- | 5''+2 | .39             | .09 | .30 |

#### Example X

Example I was repeated except that the emulsion contained 100 milligrams of the optical sensitizing dye: 3-n-butyl - 5 - (3 - ethyl - 2 - thiiazolidene ethylidene) - rhodanine. All condition of exposure were the same as those described in Example I with the following results.

| W  | B  | G  | R  | K-2   | D <sub>21</sub> | Fog | Δ   |
|----|----|----|----|-------|-----------------|-----|-----|
| 16 | -- | 10 | -- | 5''+3 | .33             | .24 | .09 |

#### Example XI

70 A gelatino silver chlorobromide emulsion was made containing about 4 mole percent excess bromide ion and 100 milligrams of the optical sensitizing dye set forth in Example V. Potassium iodide in an amount of 0.5 mole was added together with sufficient thiourea to provide 1% based on the silver halide. The exposure

conditions were the same as those in Example I with the following results.

| W  | B  | G | R  | K-2  | D <sub>21</sub> | Fog | Δ   |
|----|----|---|----|------|-----------------|-----|-----|
| 16 | -- | 4 | -- | 5'+2 | .40             | .19 | .21 |

#### Example XII

Example XI was repeated except that one mole percent of plumbous nitrate had been incorporated into the emulsion. All exposure conditions were the same as in Example I with the following results.

| W  | B  | G | R  | K-2  | D <sub>21</sub> | Fog | Δ   |
|----|----|---|----|------|-----------------|-----|-----|
| 17 | -- | 6 | -- | 5'+2 | .40             | .19 | .21 |

#### Example XIII

Example XII was repeated except that 10 mole percent of stannous chloride was added in the manner described in Example I and an excess of 64 mole percent of bromide ion was added. The exposure operations were the same as described in Example I with the following results.

| W  | B  | G  | R  | K-2  | D <sub>21</sub> | Fog | Δ   |
|----|----|----|----|------|-----------------|-----|-----|
| 19 | -- | 10 | -- | 5'+3 | .41             | .09 | .32 |

#### Example XIV

Example I was repeated except that the emulsion contained 200 milligrams of the optical sensitizing dye disclosed there instead of 100 milligrams per mole of silver halide. All conditions of exposure were the same as described in that example with the following results.

| W  | B  | G  | R  | K-2  | D <sub>21</sub> | Fog | Δ   |
|----|----|----|----|------|-----------------|-----|-----|
| 19 | -- | -- | 15 | 5'+2 | .45             | .19 | .26 |

#### Example XV

An emulsion as described in Example I but containing 160 milligrams per mole of silver halide of the optical sensitizing dye described in Example II was tested to show the effect of varying the time of latensification through the K-2 filter. The exposure and photodevelopment times and conditions remained the same as in Example I. The results are as follows:

| K-2 filter, seconds | Steps visible under white light exposure | Additional steps visible by latensification |
|---------------------|------------------------------------------|---------------------------------------------|
| 0                   | 16                                       | 0                                           |
| 2.5                 | 17                                       | +1                                          |
| 5                   | 17                                       | +1                                          |
| 10                  | 17                                       | +1                                          |
| 15                  | 17                                       | +1                                          |
| 20                  | 18                                       | +2                                          |
| 25                  | 18                                       | +2                                          |
| 30                  | 18                                       | +2                                          |
| 35                  | 18                                       | +2                                          |
| 45                  | 18                                       | +2                                          |
| 55                  | 18                                       | +2                                          |
| 60                  | 18                                       | +2                                          |
| 120                 | 17                                       | +1                                          |
| 360                 | 17                                       | +1                                          |

It will be seen that after about 60 seconds the latensifying effect begins to fall off when the above intensity for latensification is used.

#### Example XVI

The photographic element described in Example I 75

was exposed to a  $10^{-5}$  second xenon flash in the sensitometer behind a neutral density filter of 1.3 in place of the  $\sqrt{2}$  step wedge. The exposed material was then exposed for 5 and 60 seconds through a Wratten No. 47 blue filter, a Wratten No. 58 green filter or a Wratten No. 25 red filter to light of varying intensity as shown in the tables below. The material was then photodeveloped by exposing to a white fluorescent light of 40-foot candles intensity for 30 minutes. The results were determined by reading the densities on a reflection densitometer. The difference between the densities under the white light column and those under the various filters shows the improvement gained by the latensifying exposure. It will be noted that an exposure under the blue filter caused no change or a decrease in density. The sensitizing dye has a sensitivity maximum at about 6600 Å, and the tables show a consistently good improvement by latensifying through the Wratten No. 25 red filter which transmits very efficiently light above 6000 Å.

| Foot-candles of latensifying light before passing through filter | Latensification time—5 seconds |       |      |       |     |
|------------------------------------------------------------------|--------------------------------|-------|------|-------|-----|
|                                                                  | Fog                            | White | Blue | Green | Red |
| 184                                                              | .23                            | .28   | .28  | .32   | .33 |
| 63                                                               | .25                            | .36   | .32  | .36   | .38 |
| 44                                                               | .25                            | .32   | .29  | .32   | .35 |
| 30                                                               | .20                            | .33   | .32  | .35   | .37 |
| 18                                                               | .25                            | .35   | .30  | .32   | .36 |

  

| Foot-candles of latensifying light before passing through filter | Latensification time—60 seconds |       |      |       |     |
|------------------------------------------------------------------|---------------------------------|-------|------|-------|-----|
|                                                                  | Fog                             | White | Blue | Green | Red |
| 184                                                              | .21                             | .28   | .25  | .29   | .35 |
| 63                                                               | .25                             | .34   | .29  | .36   | .39 |
| 44                                                               | .22                             | .29   | .27  | .35   | .35 |
| 30                                                               | .25                             | .33   | .31  | .35   | .40 |
| 18                                                               | .23                             | .32   | .28  | .32   | .35 |

Other filters may be used for the latensifying step such as any minus blue filter and those which are minus blue and transmit efficiently, radiation in the region where the particular optical sensitizing dye confers the greatest amount of spectral response to the emulsion.

It will be seen that the process of the invention offers several advantages. By being able to latensify the latent images in the manner taught by the invention a much lower energy image exposure is possible or by the same token, a much higher effective speed is obtained from high intensity exposures. In the former case, one could for instance expose the elements to electroluminescent panels and then by the instant process produce a suitable image. In the latter case, say for oscillographic use the writing speed can be increased by about 150%. In other words the density of the image normally obtainable without latensification can be increased 100% or more.

I claim:

1. A process which comprises

- (a) exposing to image-forming radiation containing radiation in at least one of the regions of normal sensitivity of a silver halide photographic emulsion and of extended sensitivity conferred by the presence of an optical sensitizing dye, a washed, light-sensitive colloid-silver halide emulsion layer having light-developable, direct-writing characteristics and an average grain size of 0.1 to 10 microns containing
  - (1) 0.5 to 120 mole percent of a water soluble stannous salt,
  - (2) a sensitizing amount of an optical sensitizing dye taken from the group consisting of cyanine, pseudocyanine, carbocyanine and merocyanine dyes capable of extending the sensitivity of a silver bromide emulsion from the normal blue region to at least one of the green, red and infrared regions of the spectrum, and having added thereto
  - (3) at least one water-soluble halide taken from the group consisting of lithium, sodium, potas-

- sium, calcium, magnesium and ammonium chloride, bromide and iodide in an amount sufficient to provide an excess of halide ions over that necessary initially to precipitate all of the silver as silver halide,
- (b) latensifying the element resulting from the image exposure of step (a) by irradiating said element for about 1 to about 60 seconds with light radiation in the region of greatest response in the region of extra sensitivity conferred to the silver halide emulsion by said dye, and
- (c) photodeveloping the latensified element by exposing it to actinic radiation containing wavelengths from 3000 to 5000 Å, having an intensity less than the exposing radiation (a) for a period of at least one second.
- 15 2. A process according to claim 1 wherein step (c) is carried out with radiation of 50 foot-candles at a temperature of 200°-300° F.
3. A process according to claim 1 wherein the emulsion contains an orthochromatic sensitizing dye and light radiation in the green region of the spectrum is used in latensifying step (b).
- 20 4. A process according to claim 1 wherein the emulsion contains a panchromatic sensitizing dye and light radiation in the yellow region of the spectrum is used in latensifying step (b).
5. A process according to claim 1 wherein there is at least a 10% excess of halide ions present.
6. A process according to claim 1 wherein the halide ions are bromide ions.
- 25 7. A process according to claim 1 wherein the emulsion is a silver chlorobromide emulsion.
8. A process according to claim 1 wherein the emulsion

is a silver chlorobromide emulsion and the dye is 5,5'-dimethyl - 3,3',9 - triethylbenzselenazole carbocyanine iodide.

5 9. A process according to claim 1 wherein the emulsion is a silver chlorobromide emulsion and the dye is 5,5'-diphenyl-9-methyl-3,3' - diethylbenzoxazole carbocyanine iodide.

10 10. A process according to claim 1 wherein the emulsion also contains plumbous nitrate in an amount of 0.1 to 4.0 mole percent.

10 11. A process according to claim 1 wherein the emulsion layer is on a paper support.

#### References Cited by the Examiner

##### UNITED STATES PATENTS

|           |       |                |        |
|-----------|-------|----------------|--------|
| 2,843,490 | 7/58  | Jones          | 96-108 |
| 3,033,678 | 5/62  | Hunt           | 96-108 |
| 3,033,682 | 5/62  | Hunt           |        |
| 3,047,392 | 7/62  | Scott          | 96-108 |
| 3,063,350 | 11/62 | Massena        | 96-27  |
| 3,102,810 | 9/63  | Sprague et al. | 96-27  |
| 3,107,138 | 10/63 | Massena        | 96-27  |

#### OTHER REFERENCES

Sheppard: "The Optical Sensitizing of Silver Halides by Colloidal Silver," Journal of the Franklin Institute, vol. 210, No. 5, November 1930, pp. 587-608.

Clerc: "Photography Theory and Practice," 2nd edition, published by Pitman and Sons, Ltd., 1937, pp. 346 and 347 relied on.

NORMAN G. TORCHIN, *Primary Examiner.*

HAROLD H. BURSTEIN, *Examiner.*